

Patented Feb. 23, 1926.

1,574,733

# UNITED STATES PATENT OFFICE.

DAVID R. KELLOGG, OF EDGEWOOD BOROUGH, PENNSYLVANIA, ASSIGNOR TO PETERSON-KINTNER COMPANY, OF PITTSBURGH, PENNSYLVANIA, A CORPORATION OF PENNSYLVANIA.

COMPOUND FOR PROTECTING THE HANDS FROM THE EFFECTS OF CONTACT WITH OIL, GREASE, AND DIRTY SUBSTANCES.

No Drawing.

Application filed January 3, 1924. Serial No. 684,191.

To all whom it may concern:

Be it known that I, DAVID R. KELLOGG, a citizen of the United States, and a resident of the borough of Edgewood, in the county 5 of Allegheny and State of Pennsylvania, have invented a new and useful Improvement in a Compound for Protecting the Hands from the Effects of Contact with Oil, Grease, and Dirty Substances, of which the 10 following is a specification.

It is a common experience with all those who have to subject their hands to contact with oil, grease, grime and dirt in general, that the pores of their skin soon become 15 filled with particles which are very difficult, if not actually impossible, to remove without serious injury to the skin. Such particles greatly disfigure the hands. This experience is frequently had by the motorist who 20 finds it necessary to make some adjustment or repair to his motor.

It is the object of my invention to supply a means for minimizing the labor of removing such foreign substances from the skin 25 upon the completion of such work. It is essential that such result be accomplished without injury to the skin of the user. In employing the material of my invention, which will be described more fully herein, 30 the hands are first covered with a thin layer which is then rubbed well into the cracks and pores of the skin and under and around the nails. It is then allowed to dry, which action takes place in a few moments, and 35 then the hands can be used in oily dirty work without this foreign matter working into the openings of the skin. My new compound is insoluble in oils and greases and, by sealing up the cracks and pores, prevents 40 the oil, grease and dirty particles from reaching those parts. It is characteristic of my compound that when it has dried on the hands the user is scarcely conscious of its being there and no inconvenience is experienced from it in doing even the most delicate work.

While I am aware that other preparations have been used to obtain the same object as that of my invention, these have proven defective in one or more of the following respects:—

(1) Failure to keep the oil and dirt from reaching the cracks and pores.

(2) Injurious to the skin and  
(3) Make the hands unsuitable for doing 55 the work, i. e., too sticky or oily.

I have found that a mixture of clay, such as bentonite, which forms a gelatinous mixture with water, when mixed in proper proportion with a mild soap, such as Ivory 60 soap, and water, forms a paste which can be applied to the hands in the manner above described and which, when dried, protects against the effect of contact with oil, grease and grime. When the hands are so treated 65 they can be exposed to contact with oils, greases and other dirty foreign matter without damage to the skin, as all of the pores and cracks are thoroughly filled and these foreign matters prevented from lodging in 70 these openings. When the user has completed the dirty work the entire substance, i. e., the paste and the foreign matter can be washed off in water, generally without the use of any soap other than that contained in 75 the paste.

As will be apparent to those skilled in this art this material will not injure the skin.

The proportions that I have found best are bentonite 17%, Ivory soap 4½% and distilled water 78½%. I have generally preferred to add some odorous material to make the use of the compound still more pleasant. For this purpose I have found an extremely small amount of oil of peppermint or sassafras very satisfactory.

I have found it best in preparing my new compound to make separate mixtures of—

(a) Bentonite and water and

(b) Soap and water.

These two mixtures are allowed to age for a period of at least 24 hours so as to insure a thorough penetration of the water. The two pastes then formed can then be mixed and the perfuming element added. The proportions employed in each of the separate mixtures, when a paste having the consistency of that described above is desired, are bentonite 21%, water 79%, Ivory soap flakes 23.1%, hot water 76.9%. Each of these 90 should be thoroughly stirred to insure complete mixture. The compounding of these two pastes to give the final product is in the proportion of 80.7% of the bentonite paste and 19.3% of the soap paste. After 95 this mixture has been made the perfuming

element is added in sufficient amount to give the desired strength of scent.

It will be found that the paste will be too fluid and will not dry to a condition which will make its presence, on the hands of the user, unnoticed, if more than 80% of water or more than 12% of soap, or less than 10% of bentonite, is used. Again it will be found to be much less effective, being too dry and not adherent, if less than 75% of water, or 2½% of soap or more than 20% of bentonite is employed.

While the proportions given above are the preferred ones and while the materials mentioned are the ones found most suitable by me, it is not to be understood that my invention is limited to the use of them as both the proportions and the materials may be varied in ways well known to those skilled in the art without departing from the novel features of my invention.

What I claim is:

1. A compound for protecting the skin

from the effects of contact with oil, grease and dirty substances consisting of a mixture 25 of gelatinous forming clay, pure soap and water.

2. A compound for protecting the skin from the effects of contact with oil, grease and dirty substances consisting of a mixture 30 of bentonite, pure soap and water.

3. A compound consisting of a gelatinous clay, a mild soap, and water in proportions within the following limits:—gelatinous clay 10 to 20%, soap 2 to 12%, and water 75 35 to 85%.

4. A compound consisting of a bentonite, a mild soap and water in proportions within the following limits:—Bentonite 10 to 20%, soap 2 to 12%, water 75 to 85%. 40

5. A compound consisting of a mixture made up of 17% bentonite, 4.5% soap and 78.5% water.

In testimony whereof, I sign my name.

DAVID R. KELLOGG.